

# UNITED STATES PATENT OFFICE.

GEORGE EDWARD HEYL AND THOMAS THORNE BAKER, OF LONDON, ENGLAND.

## LIQUID FUEL FOR INTERNAL-COMBUSTION ENGINES.

1,171,434.

Specification of Letters Patent. Patented Feb. 15, 1916.

No Drawing.

Application filed December 8, 1914. Serial No. 876,065.

To all whom it may concern:

Be it known that we, GEORGE EDWARD HEYL and THOMAS THORNE BAKER, subjects of the King of Great Britain, residing at 5 King's House, Kingsway, London, England, have invented certain new and useful Improvements in Liquid Fuel for Internal-Combustion Engines, of which the following is a specification.

10 This invention relates to liquid fuel for internal combustion engines, and its object is to produce a liquid fuel mixture with gasolene, kerosene oil or other mineral oil liquid fuels or motor spirits, which mixture 15 provides a combined fuel vapor which is more readily ignitable than the vapor of the hydrocarbon liquid alone, whereby the vapor of a motor spirit of heavier specific gravity can be caused to ignite as readily as 20 the vapor of an ordinary motor spirit of lighter specific gravity.

The liquid fuel, according to the invention, consists of the middle distillates, which are also known as sharp oils, of coal 25 tar or analogous tars, which are distilled from tar from 170° C.-230° C., from which the naphthalene and tar acids have been almost entirely removed. These middle distillates normally contain up to 27% by 30 volume of naphthalene and about 6.5% of tar acids, such as cresols and phenols, and without treatment for the approximate removal of these substances, are not suitable for use in a fuel mixture in internal 35 combustion engines. It is therefore necessary to remove excess of naphthalene so that the liquid remains free from any deposit of naphthalene at 5° C., and becomes a substance which completely vaporizes, and 40 which burns in an internal combustion engine.

The combustion of the vaporized oil is rendered much more perfect and the formation of smoke and smell is avoided, by 45 removing the tar acids down to  $\frac{1}{2}\%$ , for instance by washing or by an ordinary neutralization process. The treated tar oils when mixed with gasolene, kerosene oil or other hydrocarbon liquid fuel for internal 50 combustion engines give a mixed vapor, which when mixed with air ignites under the action of an electric spark more readily and quicker than the separate vapors of either such tar oils or liquid fuels mixed 55 with air.

The admixture of the treated tar oils with

mineral oil, such as a petroleum oil, causes a precipitate to become deposited, and consequently with a mixture of the tar oils and a mineral oil liquid fuel the carbureter jet 60 of the engine is liable to become clogged unless the precipitate has been previously removed. Hence, unless previously precipitated from the tar oils by the admixture therewith of a moderate quantity of mineral oil, 65 the precipitate which is formed is removed from the liquid by filtration, prior to using the mixture in an internal combustion engine. The treated tar oils are preferably mixed with gasolene, kerosene oil or other 70 hydrocarbon liquid fuel in the proportions of from 25-50% of the tar oils to 75-50% of the gasolene or the like, for instance 33 $\frac{1}{3}\%$  of tar oils to 66 $\frac{2}{3}\%$  of gasolene. The mixture of treated tar oils and other mineral oil liquid fuels gives an increased mileage over ordinary motor car liquid fuels, 75 by virtue of the superior content of carbon.

A representative detailed example of the manner in which coal tar middle oil can be 80 prepared for use in a fuel mixture for internal combustion engines is as follows: Ordinary middle oil, distilled from coal tar between 170° C.-230° C., is mixed with 10-30% of caustic soda in an aqueous solution, allowed to stand and separated, and is then washed with 2-5% of sulfuric acid. The oil is then washed with water and subsequently decanted off and cooled to 4° C. When the oil has stood a sufficient period 90 for all the naphthalene which will crystallize out at this temperature to have crystallized out, the oil is either pressed out or decanted. 95

We claim:

1. A liquid fuel for internal combustion engines consisting of the middle oils of coal tar or analogous tars, from which the naphthalene and tar acids have been almost entirely removed, mixed with a mineral oil liquid fuel, and freed from deposited matter. 100

2. A liquid fuel for internal combustion engines consisting of the middle oils of coal tar or analogous tars, from which the naphthalene and tar acids have been almost entirely removed, mixed with gasolene, and freed from deposited matter. 105

3. A liquid fuel for internal combustion engines consisting of the middle oil of coal tar distilled from tar between temperatures of 170° C.-230° C., said tar being that from 110 which the naphthalene and tar acids have

been substantially removed and mixed with a mineral oil liquid fuel.

4. A fuel liquid for internal combustion engines consisting of the middle distillates of coal tar from which the naphthalene and tar acids have been almost entirely removed and a precipitate has been deposited by the addition of a moderate quantity of mineral oil and a larger quantity of mineral oil liquid mixed therewith.

5. A liquid fuel mixture for internal combustion engines consisting of the middle distillates of coal tar or analogous tars from which the naphthalene and tar acids have been almost entirely removed, such middle distillates being those containing up to 20% by volume of naphthalene and about 6.5% of tar acids, such as cresols, phenols, said naphthalene being removed from said middle distillates so that the liquid remains free from any deposits of naphthalene at 5° C., and becomes a substance which completely vaporizes and burns in an internal combustion engine, the tar acids being removed down to  $\frac{1}{2}\%$  by washing or by neutralization and a hydrocarbon liquid fuel mixed with said treated tar oils whereby a fuel is produced which when mixed with air ignites under the action of an electric

spark more readily and quicker than the vapors of either of such tar oils or liquid fuels separately.

6. A liquid fuel mixture for internal combustion engines, consisting of the middle distillates of coal tar or analogous tars from which the naphthalene and tar acids have been almost entirely removed, mixed with a mineral oil liquid fuel, the said parts being mixed in the proportions of from 25-50% of the tar oils to 75-50% of the gasoline or the like mineral oils.

7. A liquid fuel mixture for internal combustion engines, consisting of the middle distillates of coal tar or analogous tars from which the naphthalene and tar acids have been almost entirely removed and a precipitate has been deposited by the addition of a moderate quantity of mineral oil, mixed with a mineral oil liquid fuel to the proportion of 33 $\frac{1}{3}\%$  of tar oil to 66 $\frac{2}{3}\%$  of mineral oil.

In testimony whereof we affix our signatures in presence of two witnesses.

GEORGE EDWARD HEYL.  
THOMAS THORNE BAKER.

Witnesses:

R. S. SMITH,  
E. C. WALKER.